

## UNITED STATES PATENT OFFICE

2,182,815

COLOR-FORMING PHOTOGRAPHIC COM-  
POSITIONS AND PROCESSES

Edmund B. Middleton, Metuchen, and Andrew B. Jennings, New Brunswick, N. J., assignors to Du Pont Film Manufacturing Corporation, New York, N. Y., a corporation of Delaware

No Drawing. Application November 23, 1938,  
Serial No. 242,112

14 Claims. (Cl. 95—6)

This invention relates to photography. More particularly it relates to novel color-former components for use in photographic emulsions and developing processes and solutions. Still more particularly it relates to photographic elements bearing an emulsion layer which develops to form a dyed image and metallic silver in admixture therewith. The invention also pertains to processes of producing colored images.

This invention has for an object to provide new photographic color-former agents of improved spectral quality. A further object is to provide novel color-formers which couple readily upon development in colloidal emulsions to form water insoluble immobile dyes in situ with photographic images. A still further object is to provide novel color-formers which will form dyes with the oxidation products of aromatic amino developing agents or the corresponding nitroso compounds upon development of photographic images. A still further object is to provide novel color-formers which do not adversely affect the sensitivity of photographic emulsions, particularly gelatine silver halide emulsions. Still other objects will be apparent from a consideration of the herein-after described invention.

It has been formerly taught to prepare colored photographs by developing exposed silver salt emulsion layers in certain developing agents whose oxidation products are water-insoluble dyes. Thus, a silver halide layer, bearing a latent image, can be developed in an alkaline indoxyl solution, whereupon a silver image is produced alone with a blue dye image in situ with the silver. The silver image can be removed by Farmer's reducer, revealing the dye image. In like manner, a photographic record can be developed in chlor-indoxyl to produce a green image and in thio-indoxyl for a red image.

It is also known, for the purpose of preparing color pictures, to develop exposed silver halide layers by agents whose oxidation products are not colored, but which will chemically unite or couple with other organic agents, called "color-formers" to form intensely colored dyes. These "color-formers" are not photographic developers, are generally water-insoluble and produce dyes in situ with, and simultaneously with the deposition of the metallic silver image. The developers used for these proposed processes are of the diamine-aryl class, such as p-phenylenediamine or its substitution products, such as for example, di-methyl or di-ethyl p-phenylene-diamine. Color-forming compounds already proposed include,

for example, thymol, benzoyl acetone, phenacyl chloride and paranitrobenzyl cyanide.

These prior processes, however, have failed to produce colored images having the correct spectral qualities for color photography. Moreover, these prior color-formers tend to have a harmful effect on the sensitivity of silver halide emulsions, so that, for these reasons, the color-formers already known have not provided a practical means for color photography.

The above and other objects may be accomplished, and the above-described disadvantages of prior art may be obviated by the following invention which comprises the use of the cyanacetamino-bis-azoles or color-formers in photographic emulsions, solutions and processes. The color-formers contemplated by this invention have the general formula:



and



wherein A is a tetravalent aromatic hydrocarbon nucleus, and X is an atom taken from the class consisting of oxygen, sulfur, selenium and tellurium. Thus, A may be a tetravalent benzene, naphthalene, etc. nucleus in which the carbon atoms not attached to X or N may have attached thereto H, alkyl, e. g., methyl, ethyl, propyl, etc.; aryl, e. g., phenyl, tolyl, naphthyl; alkoxy, e. g., methoxy, ethoxy; halogen, e. g., chlorine, bromine, sulfonic or carboxylic acid groups.

In a preferred embodiment of the invention, A is a tetravalent 1, 2, 4, 5-benzene radical and X is oxygen or sulfur. These compounds have the following general formulae:



and



wherein X' is oxygen or sulfur and R and R' may be hydrogen, alkyl, aryl, alkoxy, halogen, sulfonic or carboxylic acid groups.

The invention will be further illustrated but is not intended to be limited by the following examples in which the parts stated are parts by weight:

EXAMPLE I

*Preparation of cyanacetamino-bis-azoles*

- The di-cyanacet derivative of 2,6-diamino-p- $\beta$ -benzobisthiazole is prepared as follows. Ethyl cyanooacetate (10 parts) is heated to 150° in an open vessel and 2.5 parts of 2,6-diamino-p- $\beta$ -benzobisthiazole are added in small portions. The temperature is maintained at 160-170° for 1/2 hour, and after cooling, the pale yellow product is filtered and washed with ether. The compound has a melting point above 270° C., is but slightly soluble in alcohol, readily soluble in glacial acetic acid, dimethyl formamide, and aqueous caustic alkali.
- 10 The 2,6-diamino-p- $\beta$ -benzobisthiazole can be prepared by reacting p-phenylene diamine hydrochloride and ammonium thiocyanate and reacting the resulting p-phenylene-bis-thiourea with bromine in a dry chlorobenzene medium and 15 heating the resulting product. The isomers and analogous compounds used as starting materials may be prepared in a similar manner.
- 15 In place of the 2,6-diamino-p- $\beta$ -benzo bis-thiazole of this example the same amount of 20 the corresponding meta compound may be used. Likewise the corresponding substituted derivatives, that is, those in which at least one hydrogen atom of the benzene nucleus is substituted by an alkyl, aryl, alkoxy, halogen, sulfonic acid 25 or carboxylic acid group may be used to form the corresponding cyanacetamino-bis-azoles. In addition to afore-specified compounds the diamino-bis-azoles of the following general formulae may be used:



30 wherein R and R' have the above significance, may be used for condensation with ethyl cyanooacetate. Similarly, the corresponding oxazoles may be used.

EXAMPLE II

- 35 A developer solution containing the following ingredients was prepared:
- Diethyl-p-phenylenediamine, hydrochloride-----grams 2
- Sodium sulfite, anhydrous-----do 5
- Sodium carbonate, anhydrous-----do 20
- Water to-----liter 1
- To which is added-----
- Dicyanacetamino-1,2,4,5-p-benzo-bis-thiazole-----gram 1.0
- Ethyl alcohol-----cubic centimeters 100
- 40 A photographic element containing an exposed silver salt image was developed in the above solution and a bluish-red and magenta dyed image of good tinctorial strength was obtained.

Similar results were obtained by the use of the following compositions:

EXAMPLE III

|                                                     |                   |     |
|-----------------------------------------------------|-------------------|-----|
| Diethyl-p-phenylenediamine hydrochloride-----       | grams             | 5   |
| Sodium sulfite, anhydrous-----                      | do                | 5   |
| Sodium carbonate anhydrous-----                     | do                | 20  |
| Water to-----                                       | liter             | 1   |
| To which is added-----                              |                   | 10  |
| Dicyanacetamino-1,2,4,5-p-benzo-bis-selenazole----- | gram              | 1.0 |
| Ethyl alcohol-----                                  | cubic centimeters | 100 |

EXAMPLE IV

|                                                   |                   |     |
|---------------------------------------------------|-------------------|-----|
| Dimethyl-p-phenylenediamine hydrochloride-----    | grams             | 15  |
| Sodium sulfite, anhydrous-----                    | do                | 5   |
| Sodium carbonate, anhydrous-----                  | do                | 20  |
| Water to-----                                     | liter             | 1   |
| To which is added-----                            |                   | 20  |
| Dicyanacetamino-1,2,4,5-p-benzo-bis-thiazole----- | gram              | 1.0 |
| Ethyl alcohol-----                                | cubic centimeters | 100 |

EXAMPLE V

To 100 ccs. of a developer having the following composition:

|                                               |                   |      |
|-----------------------------------------------|-------------------|------|
| Diethyl-p-phenylenediamine hydrochloride----- | grams             | 30   |
| Sodium sulfite (anhydrous)-----               | do                | 5    |
| Sodium carbonate (anhydrous)-----             | do                | 20   |
| Water-----                                    | cubic centimeters | 1000 |

are added from 0.1 to 1.0 gram of dicyanacetamino-1,2,4,5-p-benzo-bis-thiazole dissolved in a few ccs. of ethyl alcohol. An exposed photographic element containing exposed silver salts is then developed in aforedescribed solution.

A positive silver image which has been bleached to a silver salt image may be redeveloped in this solution. A suitable bleach may comprise a liter of water containing about 35 grams of potassium ferricyanide and 5 ccs. of 20% ammonia water. Thorough washing between treatments is essential. After color-development, the silver may be removed, leaving a pure dye image, by bleaching in ferricyanide, for example, and fixing in plain hypo.

In place of the dialkyl-substituted p-phenylenediamines set forth in the preceding examples may be substituted various other aromatic amino developing agents which have at least one unsubstituted amino group. Thus, the monoalkyl arylene diamines, such as N-ethylamino aniline, N-methylamino aniline, N-propylamino aniline, 1,4-naphthylene diamine, 4-N-diethyl naphthylamine-1, phenylene diamine as well as the salts of these bases may be used. Thus, the aromatic rings may be substituted with non-reactive groups, e.g., alkyl, aryl, ester, alkoxy and halogen groups. The salts of the bases such as the hydrochloride and sulfate are generally used because of their stability. The corresponding nitroso compounds may also be used.

The color-formers hereof are not limited in their use to developer solutions. In fact, they are preferably used in photographic emulsions. The following example illustrates this feature of the invention.

EXAMPLE VI

Ten grams of the compound prepared in Example I is dissolved in a small amount of ethyl alcohol to which is added about 50 grams of gelatin in an equal amount of water and thor-

oughly mixed. This color forming solution is then added to a liter of a silver bromide-gelatine emulsion. The emulsion is then coated upon a suitable photographic support such as paper or a cellulose derivative base, or upon another photographic emulsion which may or may not contain a different color forming dye component. After exposure in a camera or by printing through appropriate color records the photographic element may be color developed with a developing solution containing p-aminodiethylaniline to form a dyed image.

In place of the specific cyanacetamino bis-azole of this example may be substituted any of the herein described compounds of that type. Furthermore, any of the herein disclosed developing agents may be used with the latter azoles.

While it is preferred to employ silver halide-gelatin emulsions, other emulsions comprising other binding agents may be used. As examples of suitable emulsions, mention is made of collodion, gum arabic, starch and albumin emulsions, and bichromated colloid emulsions. The silver halide emulsions may contain the usual sensitizers such as the cyanine, carbocyanine, pseudo cyanine, cyazine, carbocyazine, etc. salts or bases which are used to extend the sensitivity of the photographic emulsions.

In the form of color-forming developers, the above-described compounds may also be used to re-develop bleached silver images. Thus, a silver image may be bleached in potassium ferrocyanide or a mixture of chromic and hydrobromic acids and re-exposed, whereupon the bleached image can be re-developed to silver and a dye image by the color-forming developers above described. After development, the silver is removed by any of the well known reducers such as Farmer's reducer.

Among the advantages of this invention is the fact that the colors produced are less strongly blue-absorbing than the old art compounds, which is necessary for 3-color photography, and less strongly red absorbing which is also necessary. The colors still retain the necessary high absorption of green. A further advantage resides in the fact that the resulting dyes do not migrate in emulsion layers. The color-formers are furthermore somewhat immobile.

The fact that the dye images produced according to this invention are magenta is rather surprising since a consideration of their chemical structure would lead one to suspect that they would be yellow-to-orange color formers. Thus, a new class of color formers which are distinctly different from the methyphenyl pyrazolones and have advantages thereover, is provided.

This application is a continuation-in-part of applicants' co-pending application, Serial No.

126,735, filed February 19, 1937, now Patent No. 2,140,540, issued December 20, 1938.

As many apparently widely different embodiments of this invention may be made without departing from the spirit and scope thereof, it is to be understood that we do not limit ourselves to the specific embodiments hereof except as defined by the appended claims.

We claim:

1. A color-forming photographic developer comprising an aromatic amino photographic developing agent and a dicyanacetamino bis-azole.
2. A color-forming photographic developer comprising an aromatic amino photographic developing agent and a dicyanacetamino-benzo-bis-azole.
3. A color-forming photographic emulsion comprising a light sensitive material and a dicyanoacetamino-aro-bis-azole.
4. A color-forming photographic developer comprising an aromatic amino photographic developing agent and a dicyanacetamino bis-thiazole.
5. A color-forming photographic developer comprising an arylene diamino photographic developing agent and a dicyanacetamino-benzo-bis-thiazole.
6. A color-forming photographic layer comprising a light sensitive silver halide emulsion containing a dicyanoacetamino-benzo-bis-azole.
7. A photographic element bearing a light sensitive silver halide emulsion containing a dicyanoacetamino benzo-bis-thiazole.
8. A photographic element bearing a color-forming light sensitive silver halide emulsion containing dicyanacetamino-1,2,4,5-m-benzo-bis-thiazole.
9. A photographic element bearing a color-forming light sensitive silver halide emulsion containing dicyanacetamino-1,2,4,5-p-β-benzo-bis-thiazole.
10. A process which comprises developing a photographic element bearing an emulsion containing a light sensitive material in the presence of a dicyanacetamino-aro-bis-azole.
11. A process which comprises developing a photographic element bearing an emulsion layer containing a light sensitive silver halide with an arylene diamino photographic developing agent in the presence of a dicyanacetamino-benzo-bis-thiazole.
12. As new compounds the dicyanacetamino-aro-bis-azoles.
13. As new compounds the dicyanacetamino-benzo-bis-azoles.
14. As new compounds the dicyanacetamino-benzo-bis-thiazoles.

EDMUND B. MIDDLETON.

ANDREW B. JENNINGS.

60